

Oct. 21, 1924.

1,512,560

W. E. MOORE

GEAR WHEEL

Filed Oct. 27, 1920

2 Sheets-Sheet 1

*Fig. 1.*



*Fig. 4.*



*Fig. 2.*



*Fig. 3.*



Inventor

William E. Moore,

By *Wm. L. Symons*

Attorney

Oct. 21 1924.

1,512,560

W. E. MOORE

GEAR WHEEL

Filed Oct. 27, 1920.

2 Sheets-Sheet 2

*Fig. 6.*



*Fig. 5.*



*Fig. 7.*



*Fig. 8.*



Inventor  
William E. Moore,

By  
Wm. L. Symons

Attorney

Patented Oct. 21, 1924.

1,512,560

## UNITED STATES PATENT OFFICE.

WILLIAM E. MOORE, OF BEAVER FALLS, PENNSYLVANIA, ASSIGNOR TO PITTSBURGH RESEARCH CORPORATION, A CORPORATION OF DELAWARE.

### GEAR WHEEL.

Application filed October 27, 1920. Serial No. 419,920.

To all whom it may concern:

Be it known that I, WILLIAM E. Moore, a citizen of the United States of America, residing at Beaver Falls, in the county of Beaver and State of Pennsylvania, have invented certain new and useful Improvements in Gear Wheels, of which the following is a specification.

This invention relates to gear wheels and to the process of making such wheels. My invention is also applicable to the manufacture of friction wheels and rollers, pulleys, and similar elements.

An object of my invention is the production of a wheel from a wooden blank made up of thin layers of wood cemented together, preferably with waterproof elastic cement pressure being applied during the cementing process, and while the cement is fluid, to force the cement into the pores of the wood, thoroughly permeating it, and to compress the wood to twenty-five to seventy-five per cent or less of its original thickness. Instead of waterproof cement I may use such materials as celluloid, bakelite, hard rubber or other cement which may be vulcanized into the wood.

Another object of my invention is the production of a wheel which is water and oil proof and also noiseless.

A still further object of my invention is the saturation of the wood layers with waterproof elastic cement, and then the setting of the cement while the layers are under high pressure. The layers are preferably placed with the grain of each layer crossing at an angle of 90° or less to the grain of the next layer.

It has been found that the thickness of the layers should be less than the thickness of the tooth which is formed on the periphery of the blank; otherwise I have found that the wear is increased, the strength is reduced, and there is a tendency of the wood teeth to "spawl" out between the layers.

With many classes of high-speed machinery, which are rapidly growing in number, such as machinery driven by electric motors or gasoline engines, it is desirable to use a noiseless and non-vibrating gear wheel. On electric motor drives, for instance, the jar due to metallic gear wheels is transmitted to the armature or other wires of the motor, quickly wearing out the insulation

and causing short circuits, grounds, or broken wires or parts.

Gear wheels have heretofore been made of such materials as rawhide, discs of cloth or spinnable fibre placed between metal end flanges. Wooden gear rings have also been built up of thick wooden non-compressed segments crossed and glued and held by end flanges. Such structures, however, have usually been costly or weak and non-durable and suitable only for very light service. In wheels made of comparatively thick wood held with glue, the wood is subject to expansion due to atmospheric changes and is readily damaged by absorption of oil or water. My invention does away with these objections by permeating all the pores with a waterproof elastic cement and by making the layers of very thin material, readily permeable by the cement and non-spawling.

In some cases I prefer to make up the wood disc of sector shaped pieces in layers. These sectors or "pie sections" usually have the grain running in a radial direction. The radial edges of such sections may be beveled to make them stronger than butt joints wherever such joints may appear in the gear tooth after cutting.

My invention is also applicable to crown gears and other forms of wheels. In making crown gears thin cement permeable layers are wound around the metal or other spider and the layers are compressed with a waterproof adhesive between them in the same way that spur gear wheels and other similar elements are constructed. The grain of one layer in the crown gear construction is placed radially with the grain of alternate layers placed at an angle thereto.

I have also found that material constructed in accordance with my process is a good insulator and may be used for filling discs between insulating couplings, or for insulating parts of electrical apparatus and machinery, such as terminal boards and similar devices, in which case it is sometimes desirable further to treat the block, after it has been properly formed and fitted, with a suitable varnish. After this coating has been applied, the block may be baked.

In some cases I find it is desirable to put intermediate layers between the wood layers, such layers consisting of high-strength paper, fibre, cloth, or very thin metal.

In the accompanying drawings:

Figure 1 is a plan view of a spur gear with a part broken away to show the direction of the grain of the wood;

5 Figure 2 is a section on the line 2—2 of Figure 1;

Figure 3 is a plan view of a modified form of construction of spur gear;

10 Figure 4 is an enlarged section on the line 4—4 of Figure 3;

Figure 5 is a section of a modified form of gear showing thin layers of material between the wood layers;

15 Figure 6 is a plan view of a bevel gear with a metal spider;

Figure 7 is a section on the line 7—7 of Figure 6; and

20 Figure 8 is a fragment of a section of a wheel showing the construction of a crown gear, the general construction of the wheel being the same as shown in Figure 6.

The gear illustrated in Figures 1 and 2, which is designated as a whole by the numeral 1, is made up of discs of thin layers 25 of wood or veneer 2 consisting of any suitable number, ten being shown. These thin layers may be of wood of a character having pores which may be filled by a waterproof elastic cement placed between the layers and forced into the pores of the thin layers by pressure. The layers are placed so that the grain of each layer will be at an angle of 90° or less to the grain of the next layers. In forming the blanks to construct a wheel, I prefer to use hydraulic pressure and to subject the wood to a degree of compression sufficient to cause the cement to permeate the fibres and at the same time to densify by compression the fibres to a 35 maximum degree without crushing or weakening the fibres. That is to say, the pressure applied is sufficient to compress the fibres beyond their elastic compressive strength and to increase the number of fibres per unit thickness but not great enough to 40 compress the fibres until they become a pulp and also not great enough to reduce materially the strength of the fibres. The layers are then held under pressure while the cement hardens. I do not, however, limit my 45 invention to a highly compressed blank, but may use any degree of compression that seems desirable under the circumstances, and may use a vacuum press or air or fluid 50 pressure to cause the compression and to fill the pores of the wood with the cement.

55 After the adhesive has vulcanized or set and the blank has hardened, the necessary opening 3 for a shaft may be made, a metal hub 4 may be attached, as shown, in any suitable manner, as by rivets or bolts 5, and metal flanges 6 may be attached by rivets or bolts 7. These flanges may be attached before the teeth 8 are cut. The teeth are 60 cut by any of the well known means of cut-

ting gear teeth through the metal and the layers of wood.

In Figure 5 is illustrated the use of material between the layers of wood. Each layer is shown as having between it and the adjacent layer a thin layer 9 of high-strength paper, fibre, cloth, or very thin metal.

In Figures 3 and 4 a gear wheel of a slightly modified construction is shown. 75 This wheel is made up of six "pie-shaped" sectors 10 having the grain generally radial, but the sectors are so arranged that the grain of each layer is at an angle to the adjacent layer. These sectors are beveled as 80 shown at 11 in Figure 4, and the joints are staggered in order to strengthen the structure. This form of wheel has the usual hub and end flanges.

In Figures 6 and 7 the construction of a 85 bevel gear in accordance with my invention is illustrated. In this form of wheel a metal spider 12 of the ordinary construction is used. Around the periphery 13 of this spider are placed a suitable number of 90 thin layers of wood 14, seven being shown. The grain of the wood in each layer is placed at an angle to the grain of the wood in an adjoining layer. It is found preferable to have the grain of the wood generally vertical. Around the outer layer is placed a 95 metal band 15. The layers and outer metal band are attached to the wheel by any suitable means, such as bolts or rivets 16.

In Figure 8 the construction of a crown 100 gear is shown. This structure is identical with the construction of a bevel gear, except in the shape of the tooth portion 17, which is similar to the tooth of the spur gear.

105 I claim:

1. The process of producing a gear blank comprising superimposing thin layers of wood, placing a cement between said layers, applying sufficient pressure to change the 110 thickness of said layers to approximately twenty-five per cent of the original thickness of the layers and to force said cement into the pores of the wood of said layers and continuing said pressure until the cement 115 "sets".

2. A gear wheel comprising thin layers of wood, said layers being held together by waterproof elastic cement, said layers having the pores thereof saturated with said 120 cement and said layers being reduced by compression to approximately twenty-five per cent of their original thickness.

3. A gear wheel comprising thin layers of wood, said layers being held together by 125 waterproof elastic cement, said layers having the pores thereof saturated with said cement and said layers being reduced by compression to approximately twenty-five per cent of their original thickness and said 130

gear wheel having teeth thereon greater in thickness than the thickness of the layers of wood from which said gear wheel is made.

4. The process of producing a gear blank comprising superimposing thin layers of wood, placing a cement between said layers, applying sufficient pressure to compress the fibres of the layers beyond their elastic compressive strength and to increase the number of fibres per unit thickness without compressing the fibres sufficiently to reduce their strength materially and to reduce them to a pulp and to force said cement into the pores of said layers of wood and continuing said pressure until the cement "sets".

5. A gear wheel comprising thin layers of wood, said layers being held together by waterproof elastic cement, said layers having the pores thereof saturated with said cement, and said layers being reduced by compression until the fibres thereof have been compressed beyond their elastic compressive strength and until the number of fibres per unit thickness has increased and without compressing the fibres to a pulp and without reducing the strength of the fibres materially. 20 25

In testimony whereof I affix my signature.

WILLIAM E. MOORE.